

## UNITED STATES PATENT OFFICE

2,687,376

## RUST-PREVENTIVE COMPOSITIONS

John D. Spivack, Bayonne, N. J., assignor to Tide  
Water Associated Oil Company, Bayonne, N. J.,  
a corporation of Delaware

No Drawing. Application September 13, 1951,  
Serial No. 246,513

14 Claims. (Cl. 252—51.5)

1

The present invention relates to rust-inhibiting compositions and, particularly, to compositions adapted for prevention of rusting of corrosion-prone metals upon exposure thereof to corrosion-inducing conditions.

Broadly speaking, the compositions embodied herein comprise a suitable vehicle and a small amount, sufficient to impart rust-preventive characteristics thereto, of a novel di-nitrogen-containing dicarboxylic acid as described more fully hereinafter.

With reference to the vehicle component of the compositions embodied herein, materials may be employed which, though otherwise suitable for a particular usage, may require improvement with respect to their ability to prevent rusting of metals in contact therewith and exposed to rust-inducing conditions such as highly humid atmospheres. For purposes of illustration but not limitation, the vehicle may be of the volatile or non-volatile type of hydrocarbons, such as mineral oils and fractions thereof, examples of which include hydrocarbon lubricating oils, greases, petrolatum, and the like. Thus, and depending on intended usage of the novel compositions, the vehicle component thereof may be a material having properties suitable for such usage except for desired improvement in rust-preventive characteristics and is capable of being improved therein by a rust-inhibiting agent as embodied herein. Hence, compositions embodied herein include those contemplated for use as hydraulic fluids, slushing compositions, lubricants, and the like and, in particular, liquid compositions contemplated for use in lubrication of turbines exposed to severe rust-inducing conditions.

The di-nitrogen-containing dicarboxylic acids embodied for use herein as the rust-inhibiting component, are dimer products definable as di(N-carboxyalkyl alkanamides) and described in my copending application Serial No. 231,891, filed June 15, 1951, now U. S. Patent No. 2,644,826, issued July 7, 1953. As set forth in said copending application, the disclosure of which is incorporated by reference herein, a method by which di(N-carboxyalkyl alkanamides) contemplated for use herein may suitably be prepared comprises subjecting a (N-alkanoyl)iminodialkanoylnitrile to basic hydrolysis in the presence of a suitable hydroxyllic liquid under ammonia-liberating reaction conditions. In such preparation of the novel rust-inhibiting alkanamides, the (N-alkanoyl)iminodialkanoylnitrile employed as the reactant may vary over a wide range of carbon atom content with respect to

2

the alkanoyl radical in the (N-alkanoyl) grouping and, as used herein, the term alkanoyl is intended to include the acyl residue of fatty acids both of the saturated and unsaturated type. For purposes of illustration and not limitation, (N-alkanoyl)iminodialkanoylnitriles that may be employed for preparation of the novel rust-inhibiting agent may contain, as the alkanoyl radical in the (N-alkanoyl) grouping, an acyl residue of a long chain fatty acid, e. g. containing about six to about thirty carbon atoms, such as the acyl residue from stearic acid, oleic acid, behenic acid, caprylic acid, and the like. Examples of such (N-alkanoyl)iminodialkanoylnitriles include the (N-alkanoyl)iminodipropionitriles and, more specifically, nitriles such as (N-stearoyl)iminodipropionitrile, (N - lauroyl)iminodipropionitrile, (N - behenoyl)iminodipropionitrile, (N - capryloyl)iminodipropionitrile, and the like.

The di(N-carboxyalkyl alkanamides) possess such highly effective rust-preventive characteristics that usually only a small amount thereof is required for preparation of the compositions embodied herein. Hence, highly effective rust-preventive compositions may be prepared comprising the vehicle in major amount by weight and a minor amount of the rust-inhibiting agent. The actual amount of rust-inhibiting agent employed may be varied depending on factors such as the desired degree of improvement in rust-preventive characteristics, solubility characteristics of the rust-inhibiting agents in the particular vehicle employed, and the like but, for most purposes, the rust-inhibiting agent is employed in about 0.005 to about 1% by weight based on the weight of the composition. Although the compositions embodied herein comprise, in broad aspect, a vehicle capable of being imparted with rust-preventive properties by having dissolved therein a rust-inhibiting di(N-carboxyalkyl alkanamide), an embodiment relates to such compositions which also contain a solubilizing agent for the di(N-carboxyalkyl alkanamides). For example, certain of the di(N-carboxyalkyl alkanamides) are slightly, if at all, soluble in certain vehicles and, in instances wherein it is desired to prepare rust-inhibiting solutions containing the aforescribed alkanamides in such vehicles, a solubilizing agent that is compatible with the vehicle and functions as a solubilizing agent for the alkanamide is employed. In illustration of such an embodiment, certain of the di(N-carboxyalkyl alkanamides) possess limited solubility in paraffinic-type oils, such as highly refined conventional solvent extracted lubricating

oils useful for lubrication of turbines, and in the use thereof for preparation of compositions as embodied herein a solubilizing agent for the alkanamide is also incorporated in the composition. Illustrations of suitable solubilizing agents for such usage includes oil-soluble alkylamines such as the amylamines, octadecylamines, primary long chain branched alkyl amines, and the like.

In order to further describe the invention, the following examples set forth compositions illustrative but not limitative of this invention; and included therein are the performance characteristics of the compositions when subjected to the severe rust-inducing conditions of the corrosion test described in Navy Department specification pamphlet 14-0-15, symbol 2190-T, as amended March 1, 1948, relating to specifications for steam turbine lubricants. Briefly, the test described therein provides that polished cylindrical steel specimens be partially immersed for 48 hours in a bath maintained at 140° F. and composed of 300 ml. of the lubricant under test and 30 ml. of synthetic sea water. In order to pass that test, the immersed portions of the steel specimens must show no corrosion at the completion of the 48-hour period. For purposes of completeness, the following procedure is also set forth illustrative of a suitable method for preparation of the di(N-carboxyalkylalkanamides) employed in preparation of the rust-inhibiting agents used in the compositions of the examples hereinafter set forth.

#### PREPARATIONS OF DI(N-CARBOXYETHYLALKANAMIDES)

##### A. Preparation of di(N-carboxyethylstearamide)

Nine grams (0.023 mole) of (N-stearoyl)-iminodipropionitrile were introduced into a 300 ml. round-bottom flask containing a solution of 15 grams of potassium hydroxide in 150 cc. of n-propanol. The flask was connected to a reflux condenser through an adapter providing for sweeping the inside of the flask with dry nitrogen and the condenser connected to an absorber (standard aqueous  $H_2SO_4$ ) to absorb liberated ammonia. The reaction mixture was maintained at reflux temperature of the propanol until substantially two moles of ammonia were absorbed for each mole of nitrile reacted. The time of reaction was 1 $\frac{1}{4}$  hours and the amount of ammonia absorbed was 42.9 millimoles. The refluxed product was a homogeneous solution containing the potassium salts of di(N-carboxyethylstearamide). The solution was poured into 400 cc. of water and the resultant solution acidified with hydrochloric acid to convert the potassium salts to the free acids which precipitated as a white gelatinous mass that was filtered, air dried and crystallized from acetone. The crystallized product had a melting point of 119-120° C., possessed two carboxyl groups per molecule evidenced by neutralization equivalent points of 708 and 352 upon determination thereof electrometrically in dimethylformamide and possessed two nitrogen atoms per molecule. The di-nitrogen-containing dicarboxylic acid product thus produced and herein designated di(N-carboxyethylstearamide) had an empirical formula of  $C_{42}H_{80}O_6N_2$  and carbon, hydrogen and nitrogen content as shown in the following tabulation which also includes corresponding theoretical values for the di(N-carboxyethylstearamide) derivative from (N-stearoyl)iminodipropionitrile.

|                           | Reaction Product | Theoretical Values for di(N-carboxyethyl stearamide) |
|---------------------------|------------------|------------------------------------------------------|
| Carbon Content            | 71.16%; 71.34%   | 71.11%                                               |
| Hydrogen Content          | 11.80%; 11.38%   | 11.37%                                               |
| Nitrogen Content          | 4.46%; 4.63%     | 3.95%                                                |
| Neutralization Equivalent | 708 and 352      | 709.1 and 354.6.                                     |

##### B. Preparation of di(N-carboxyethylstearamide)

By use of a procedure as described hereinbefore using a 0.43 Normal ethylene glycol-KOH solution instead of n-propanol in the reaction, the corresponding derivative from (N-lauroyl)-iminodipropionitrile was prepared, said derivative being termed di(N-carboxyethylstearamide) and characterized by being a white crystalline material having a melting point of 109-111° C.

##### Example I

A solution was prepared comprising (by weight) 0.05% of di(N-carboxyethylstearamide) and 0.03% of diethylamine as a solubilizing agent in a light turbine oil prepared by solvent (furan) extraction of a predominantly paraffinic distillate lube and which oil per se is substantially ineffective in protecting metals against rusting under the conditions of the aforescribed corrosion test. Another composition was prepared comprising by weight 0.08% of di(N-carboxyethylstearamide) and 0.048% of di-n-amylamine in the aforesaid light turbine oil.

Both of the compositions of this example were subjected to the aforescribed corrosion test and performed effectively as rust-preventive compositions in the presence of synthetic sea water as no evidence of corrosion on the polished steel specimen had occurred in the 48-hour immersion test.

##### Example II

A solution was prepared comprising (by weight) 0.03% of di(N-carboxyethylstearamide) and 0.036% of "Alkylamine JM" as a solubilizing agent in the aforescribed light turbine oil. "Alkylamine JM" is a product marketed by the Rohm and Haas Company of Philadelphia, Pa., and understood to comprise an 18 carbon atom primary branched chain alkylamine which, when used alone in a turbine oil as aforesaid and subjected to the conditions of the aforescribed test, fails to substantially (if at all) improve the rust-preventive characteristics of the turbine oil.

Another solution was prepared comprising (by weight) 0.05% of di(N-carboxyethylstearamide) and 0.06% of "Alkylamine JM" in the aforescribed turbine oil.

Both of the compositions of this example, upon being subjected to the conditions of the aforescribed corrosion test, protected the metal specimens against corrosion during the 48-hour exposure.

Although the present invention has been described in conjunction with certain preferred embodiments thereof, those skilled in the art will readily recognize that variations and modifications can be made. Moreover, it should be understood that compositions, as embodied herein and containing the aforescribed rust-inhibiting agent, may also contain additional ingredients for imparting other desired properties to the composition. In illustration, the compositions may contain an anti-oxidant, such as an aromatic amine anti-oxidant, e. g. phenyl alpha naphthylamine,

viscosity index improvers, e. g. polyacrylates, antifoam agents of the silicone type, and the like.

I claim:

1. A composition comprising a substantially non-corrosive vehicle in major amount based on the weight of the composition and a small amount, sufficient to impart rust-inhibiting properties, of a rust-inhibiting di(N-carboxyalkyl-alkanamide) in which the alkanoyl radical of the alkanamide grouping is an alkanoyl residue of a long chain fatty acid.

2. A composition, as defined in claim 1, wherein the vehicle is a hydrocarbon.

3. A composition, as defined in claim 1, wherein the vehicle is a mineral oil.

4. A composition, as defined in claim 1, wherein the alkanamide is a di(N-carboxyethylalkanamide).

5. A composition, as defined in claim 1, wherein the alkanamide is characterized by containing, in the alkanoyl radical of the alkanamide grouping, an alkanoyl residue of a fatty acid of about six to about thirty carbon atoms.

6. A composition, as defined in claim 1, which in addition contains a solubilizing agent for the alkanamide.

7. A composition comprising a hydrocarbon vehicle in major amount, based on the weight of the composition, having dissolved therein a small amount, sufficient to impart rust-preventive characteristics, of a rust-preventive di(N-carboxyethylalkanamide) in which the alkanoyl radical of the alkanamide grouping is an alkanoyl residue of a long chain fatty acid.

8. A composition, as defined in claim 7, wherein

the alkanamide contains, as the alkanoyl radical of the alkanamide grouping, an alkanoyl residue of a fatty acid of about six to about thirty carbon atoms.

5 9. A composition, as defined in claim 7, which, in addition, contains an oil-soluble solubilizing agent for the alkanamide.

10. A composition, as defined in claim 9, wherein the solubilizing agent is a member from the group consisting of oil-soluble primary alkylamines and oil-soluble secondary alkylamines.

11. A composition, as defined in claim 7, wherein the vehicle is a mineral oil of turbine lubricating grade.

15 12. A composition comprising a mineral oil of lubricating grade in major amount based on the weight of the composition having dissolved therein a small amount, sufficient to impart rust-preventive characteristics to said composition, of a di(N-carboxyalkylalkanamide) from the group consisting of di(N-carboxyethyl stearamide) and di(N-carboxyethyl lauramide).

13. A composition, as defined in claim 12, which, in addition, contains an oil-soluble alkylamine as a solubilizing agent for said di(N-carboxyalkylalkanamide).

20 14. A composition, as defined in claim 12, wherein the mineral oil is a solvent refined mineral oil of turbine lubricating grade.

References Cited in the file of this patent

UNITED STATES PATENTS

| Number       | Name    | Date          |
|--------------|---------|---------------|
| 35 2,388,132 | Fischer | Oct. 30, 1945 |
| 30 2,403,067 | Fischer | July 2, 1946  |